

## UNITED STATES PATENT OFFICE.

GUILLAUME JUSTINE KROLL, OF LUXEMBURG, LUXEMBURG.

## PROCESS FOR THE SEPARATION AND RECOVERY OF METALS FROM METAL ALLOYS.

No Drawing.

Application filed September 21, 1920. Serial No. 411,751.

*To all whom it may concern:*

Be it known that I, GUILLAUME JUSTINE KROLL, metallurgical engineer, a subject of the Grand Duchess of Luxemburg, residing at Rue Schmilz-Hollerich 52, Luxemburg, Grand Duchy of Luxemburg, have invented certain new and useful Improvements in Processes for the Separation and Recovery of Metals from Metal Alloys, of which the following is a specification.

The present invention relates to a process for the purpose of separating individual constituents from metal alloys (including impure metals) in order either to free the metal alloys from the injurious metallic constituents contained therein, or to recover the eliminated constituents.

The invention is based on the observation that when alkaline-earth metals (including magnesium) are introduced into fused metal alloys they combine with certain metals of the alloy under treatment to form alloys or other compounds or mixtures which, inasmuch as they have a different fusing point and a different specific gravity from the remaining part of the alloy under treatment, can be easily separated from the latter by known methods.

Accordingly, the present invention consists in introducing alkaline-earth metals, or alloys (mixtures) of said metals between themselves or with other metals, into the fused metal alloys under treatment. The separable alloys or other compounds or mixtures above mentioned are thereby formed within the metal alloys, and separate from the remaining part of the metal alloy under treatment by stratification either immediately or after cooling; or if they remain distributed throughout the mass of the metal, they may be separated out by one or more segregation or liquation processes or by crystallization or otherwise.

To mention a few examples, it is possible to separate antimony, bismuth, arsenic, tellurium (in a less easy manner, also tin, copper, zinc and the noble metals) from lead alloys, by introducing sodium, calcium, strontium, barium or magnesium. Antimony, arsenic and bismuth, may be separated from alloys of tin; antimony, arsenic, tin, and tellurium from alloys which mainly contain bismuth; antimony and arsenic from alloys of zinc in the same manner.

The choice of the alkaline-earth metal to

be used depends on the kind of the metal alloy and on the constituents which have to be separated out therefrom. Calcium is, in general, the most efficient alkali earth metal for carrying out the present invention.

The alkali metals and the rare earth metals act in a similar manner as the alkali earth metals. It may be advantageous in the present method to use the alkali earth metals or the rare earth metals in combination with alkali metals. This can be effected by using an alloy (mixture) of alkali earth metals and alkali metals or rare earth metals. It may also be preferable to first cause the alkali earth metals or metal (such as calcium) to act upon the metal alloy under treatment in order to remove part of the constituents to be separated, and subsequently cause the alkali metals or metal (such as sodium) or the rare earth metals to act upon the remaining part of the metal alloy under treatment in order to remove the remaining constituents to be separated, or these subsequent operations may be effected vice versa.

It is obvious that the alkaline-earth metal or alkali metal or rare earth metal may also be added to the metal alloy under treatment in any other form, for example in the form of an alloy, or they may be incorporated into the metal alloy under treatment by electrolysis or a chemical process.

For carrying out the process it is, of course, unnecessary to add the required amount of alkaline-earth metal (or alkali metal or rare earth metal) in one portion; but the treatment may be effected in a series of successive working stages with successive portions of the required amounts of alkaline-earth metals (or alkali or rare earth metals.) In these successive operations different alkali earth metals may be made use of.

*Example 1.*—5% of calcium have been alloyed into a fused alloy of tin containing 5% antimony and the resulting metal mixture was slowly cooled and solidified. The lower and upper part of the metal regulus were analyzed separately. The upper part gave 9.45% antimony and the lower part 0.20% antimony.

*Example 2.*—Lead containing 0.2% of bismuth has been treated in a fused state with 0.2% of calcium. After slowly cooling down to its solidification point, the alloy was sub-

60

65

70

75

80

85

90

95

100

105

110

mitted to a liquation process. The effluent part of the metal contained 0.04% bismuth, whilst the residue showed 4% bismuth.

*Example 3.*—Hard lead containing 12% of antimony has been first treated with 4% of its weight of sodium. A liquid mass raised to the surface of the metal bath and was skimmed off. This mass contained 65% antimony, while the antimony content of the 10 remaining lead has been lowered to 1.5%. By a second similar treatment with calcium the antimony content of the lead was reduced to traces, while the lead contained yet 0.26% of bismuth. This lead was treated 15 with 0.3% calcium. A more or less solidified mass raised to the surface of the metal bath and was skimmed off. The analysis of this mass showed 2.0% of bismuth, while in the remaining lead the bismuth content was reduced 20 to 0.049%.

What I claim as new and desire to secure by Letters Patent of the United States is:

1. The method of separating and recovering metallic constituents from metal alloys (including impure metals), which comprises introducing an alkali-earth metal (including magnesium) into said metal alloys, forming thereby a compound of the alkali-earth metal with the metallic constituents to be separated, this compound having a different melting point from and a specific gravity not more than that of the main metal, and eliminating this compound from the remaining part of the metal alloy under treatment. 30

35 2. The method of separating and recovering metallic constituents from metal alloys (including impure metals), which comprises introducing a plurality of alkali-earth metals (including magnesium) into said metal alloys, forming thereby a compound of the alkali earth metals with the metallic constituents to be separated, this compound having a different melting point from and a specific gravity not more than that of the main metal, and eliminating this compound from the remaining part of the metal alloy under treatment. 45

50 3. The method of separating and recovering metallic constituents from metal alloys (including impure metals), which comprises introducing an alloy (mixture) of one or more alkali-earth metals (including magnesium) with other metals into said metal alloy forming thereby a compound of the alkali earth metals with the metallic constituents to be separated, this compound having a different melting point from and a specific gravity not more than that of the main metal, and eliminating this compound from the remaining part of the metal alloy under treatment. 55

60 4. The method of separating and recovering metallic constituents from metal alloys (including impure metals), which comprises introducing calcium into said metal alloys, 65

forming thereby a compound of calcium with the metallic constituents to be separated, this compound having a different melting point from and a specific gravity not more than that of the main metal, and eliminating this compound from the remaining part of the metal alloy under treatment. 70

5. The method of separating and recovering metallic impurities from impure lead, which comprises introducing calcium into the impure 75 lead, forming thereby a compound of calcium and bismuth, this compound having a different melting point from and a specific gravity not more than that of the main metal, and eliminating said compound from the lead under treatment. 80

6. The method of separating and recovering bismuth from impure lead, which comprises introducing calcium into the impure 85 lead, forming thereby a compound of calcium and bismuth, this compound having a different melting point from and a specific gravity not more than that of the main metal, and eliminating said compound from the lead under treatment. 90

7. The method of separating and recovering bismuth from impure lead, which comprises introducing an alloy (mixture) of calcium with other metals into the impure 95 lead, forming thereby a compound of calcium and bismuth, this compound having a different melting point from and a specific gravity not more than that of the main metal, and eliminating said compound from the lead under treatment. 100

8. The method of separating and recovering metallic constituents from metal alloys (including impure metals), which comprises introducing an alloy (mixture) containing alkali-earth metals (including magnesium) and alkali metals into said metal alloy, forming thereby a compound of the alkali-earth metals and alkali metals with the metallic constituents to be separated, this compound having a different melting point from and a specific gravity not more than that of the main metal, and eliminating this compound from the remaining part of the metal alloy under treatment. 115

9. The method of separating and recovering subsequently metallic constituents from metal alloys (including impure metals) which comprises introducing an alkali metal into said metal alloys, forming thereby a compound of the alkali metal with one or more of the metallic constituents to be separated, eliminating this compound from the remaining part of the metal alloy under treatment, introducing an alkali-earth metal (including magnesium) into the remaining part of the metal alloy under treatment, forming thereby a compound of the alkali-earth metal with the remaining part of the metallic constituents to be separated, and 120

eliminating this compound from the remaining part of the metal alloy under treatment the compounds being eliminated having a different melting point from and a specific gravity not greater than that of the main metal.

10. The method of separating and recovering subsequently metallic impurities from impure lead, which comprises introducing sodium into the impure lead, forming thereby a compound of sodium with part of the metallic impurities to be separated, eliminating this compound from the remaining part of the lead under treatment, introducing calcium into this remaining part of the lead under treatment, forming thereby a compound of calcium with the remaining part of the metallic impurities to be separated, and eliminating this compound from the remaining part of the lead under treatment the compounds being eliminated having a different melting point from and a specific gravity not greater than that of the main metal.
15. 11. The method of separating and recovering metallic constituents from metal alloys (including impure metals), which comprises introducing an alloy (mixture) containing alkali-earth metals, (including magnesium) and rare earth metals into said metal alloy, forming thereby a compound of the alkali-earth metals and rare earth metals with the metallic constituents to be separated, and eliminating this compound from the remaining part of the metal alloy under treatment.
20. 12. The method of separating and recovering subsequently metallic constituents

from metal alloys (including impure metals) which comprises introducing an alkali-earth metal (including magnesium) into said metal alloys, forming thereby a compound of the alkali-earth metal with one or more of the metallic constituents to be separated, eliminating this compound from the remaining part of the metal alloy under treatment, introducing rare earth metals into the remaining part of the metal alloy under treatment, forming thereby a compound of the rare earth metals with the remaining part of the metallic constituents to be separated, and eliminating this compound from the remaining part of the metal alloy under treatment.

13. The method of separating and recovering subsequently metallic impurities from impure lead, which comprises introducing calcium into the impure lead, forming thereby a compound of calcium with part of the metallic impurities to be separated, eliminating this compound from the remaining part of the lead under treatment, introducing rare earth metals into this remaining part of the lead under treatment, forming thereby a compound of the rare earth metals with the remaining part of the metallic impurities to be separated, and eliminating this compound from the remaining part of the lead under treatment.

In testimony whereof I affix my signature in presence of two witnesses.

GUILLAUME JUSTINE KROLL.

Witnesses:

V. MULLER,  
R. HENPEN.